

Oct. 13, 1925.

1,556,820

H. HOCKING

MANUFACTURING RED LEAD

Filed Aug. 5, 1924



Inventor:  
Henry Hocking  
By *[Signature]*  
James Daniels  
Attorney

## UNITED STATES PATENT OFFICE.

HENRY HOCKING, OF BUDAPEST, HUNGARY, ASSIGNOR OF ONE-HALF TO ORION REZ-KOHO-ES RÉZGÁLICGYÁR RÉSZVÉNYTÁRSASÁG, OF BUDAPEST, HUNGARY.

## MANUFACTURING RED LEAD.

Application filed August 5, 1924. Serial No. 730,298.

To all whom it may concern:

Be it known that I, HENRY HOCKING, a subject of the King of Great Britain, residing at Budapest, Hungary, have invented 5 certain new and useful Improvements in Manufacturing Red Lead, of which the following is a specification.

My invention relates to an improved process for manufacturing red lead in a single operation from metallic lead.

The difficulties in carrying out the old processes of this kind in a manner satisfying practical requirements arise from the fact that when oxidizing metallic lead, the layer 15 or incrustation of oxide produced on the surface of the metallic lead particles prevents such particles from being oxidized or at least retards considerably the oxidizing process.

Now, in order to overcome the said difficulties, in practice special means are usually applied adapted to stir or cut the bath of liquid lead during oxidation whereby constantly new surfaces of metallic lead are exposed and subjected to the direct action of the oxidizing gases.

The lead-oxide produced in this way, however, generally constitutes a leafy mass still containing considerable quantities of metallic lead which mass is not suitable for homogeneously oxidizing further to the second stage to get red lead of marketable quality, but has to be prepared for the said second oxidizing stage in a special way by applying first a separate milling or grinding, and then a separate washing operation to convert the leafy lead-oxide mass into a fine powder free from lead particles.

Now, according to my invention marketable red lead of high quality may be obtained from metallic lead by a single operation satisfying all requirements as to economy and output. This is accomplished by oxidizing metallic lead heated under pressure to a temperature above its melting point through the action of oxidizing gases while it is simultaneously subjected to a milling or grinding action.

Owing to the simultaneous and combined 50 oxidizing action under pressure and milling or grinding the material while it is being oxidized, the formation of surface oxide incrustation on metallic lead particles becomes practically or wholly impossible because any oxide formed is almost instanta-

neously crushed to powder sufficiently fine to be immediately oxidized to the second stage resulting in the formation of red lead. Moreover, owing to the continuous milling or grinding acting upon the material while it is being oxidized the red lead is attained directly from the oven in a highly divided powdered form not requiring any separate subsequent operation to get a commercial quality of marketable red lead.

I am aware of the fact that it is well known per se to roast lead-oxide or white lead to red lead under pressure. This way, however but the second stage of oxidizing lead may be carried out which starts 60 from lead-oxide or white lead previously brought to a powdered form by means of a separate grinding operation and then freed from metallic lead particles by a separate washing operation following the grinding 65 whereas according to my invention metallic lead may be converted to red lead directly without separate grinding and washing operations between the two oxidizing stages 70 as heretofore found generally necessary.

My invention will be readily understood from the following description taken in connection with the accompanying drawing in which Figure 1 is a vertical cross section showing apparatus in which my invention 75 can be carried into effect, the section being taken on line 1—1 in Figure 2, and Figure 2 is a vertical longitudinal section taken on line 2—2 in Figure 1.

My apparatus consists of a ball mill *a* 80 provided with hollow axial projecting shafts *b* rotatably mounted within the combustion chamber of a furnace *c*. One of the hollow axial projections *b* is provided with a fluid tight cover *d* and serves as a channel for 85 admitting a charge to the mill while the other hollow axial projection *b* communicates with a pipe *e* detachably connected to a convenient source *k* of oxidizing gas such as air, or the like under pressure.

As grinding means I prefer to use iron balls *g* although any other form of rolling bodies may be used if found desirable.

To enable the ball mill *a* to be rotated a pulley *f* is provided on one of the axial projections *b*, said pulley being connected to any convenient kind of power (not shown).

The operation is as follows:

The ball mill is charged through the channel *b* with solid or melted metallic lead 110

whereupon the said channel is closed by means of the cover *d*. The mill is then rotated by the pulley *f* and oxidizing gas under pressure is admitted. Within the ball mill I prefer to maintain a pressure of about 4 to 6 atm., and should the pressure for any reason, chemical binding or leakiness for instance, fall below this I raise the pressure again by admitting an additional supply of the oxidizing gas. The heating of the exterior of the ball mill is regulated in such a manner that the charge therein is heated to a temperature above the melting point of metallic lead, preferably to about 300-350° C. In continuing the operation as described for about five hours the metallic lead is oxidized to red lead in finely divided powdered form.

It is believed that in comparison with the known two stage processes the single stage process according to my invention will result in a considerable saving of cost and time. The two stage processes as a rule require, inclusive of the separate grinding and washing operations, 144 working hours, as well as a considerable number of workmen to carry out the different operations at different places and in different machines, whereas the process according to my invention will require but five hours to produce directly from metallic lead, marketable red lead, the handling of the material being limited to the charging and discharging of the ball mill, and the necessity for transporting intermediate products to different furnaces and machine as heretofore will be obviated. As a further result thereof the

costs of the whole plant will be considerably smaller than those for the two stage processes. The amount of fuel necessary to oxidize metallic lead to red lead will be a mere fraction of the fuel used with known processes, and the chemical reaction will go on without any loss whatever and practically with quantitative yield. A further advantage resulting from my one stage process is that workmen will not be subjected to the danger of lead poisoning since the lead charge is enclosed in one and the same hermetically sealed chamber until completely oxidized to red lead.

Although I have described my apparatus in connection with my one stage process for making red lead, it is obvious that I may charge my ball mill if desired with lead oxide or white lead to which will also be converted to red lead in powdered form if subjected to the simultaneous and combined milling and pressure heating actions.

What I claim is:—

The process of making red lead which comprises enclosing lead containing material in a pressure tight vessel, simultaneously enclosing in the said vessel rolling bodies made of material the melting point of which is considerably higher than that of lead, maintaining within the said vessel a raised pressure by means of an oxidizing gas under pressure, and rotating the said vessel while the charge therein is being heated to a temperature above the melting point of lead.

In testimony whereof I affix my signature.

HENRY HOCKING.